

1

3,793,419

**PROCESS FOR THE MANUFACTURE OF VISCOSE FIBRES WITH NOVEL DYEING PROPERTIES**

Felix Steinlin, Dornach, Soleure, and Horst Nobs, Magden, Aargau, Switzerland, assignors to Ciba-Geigy AG, Basel, Switzerland

No Drawing. Continuation of abandoned application Ser. No. 858,138, Sept. 15, 1969. This application Jan. 31, 1972, Ser. No. 222,319

Claims priority, application Switzerland, Oct. 1, 1968, 14,660/68

Int. Cl. D01f 3/12

U.S. Cl. 264—78

8 Claims

**ABSTRACT OF THE DISCLOSURE**

A process is provided for the manufacture of viscose fibres with improved dyeing properties. In this process a polyamine-amide from (a) a higher unsaturated fatty acid or its dimer or polymer and (b) a polyalkylene-polyamine and a further reaction product of (c) a polyepoxide compound and (d) a stoichiometric excess of a polyalkylene-polyamine are incorporated into the viscose spinning solution in a finely divided form from which spinning solution the viscose being thereafter precipitated and shaped.

The fibres obtained show a good receptivity for dyestuffs suitable for dyeing cellulose materials and also for acid wool dyestuffs and dispersion dyestuffs.

This is a continuation of application Ser. No. 858,138 filed on Sept. 15, 1969 and now abandoned.

The present invention relates to a process for the manufacture of viscose fibres having novel dyeing properties. According to the present invention there is provided a process for the manufacture of viscose fibres which comprises adding to the viscose spinning solution before precipitation of a polyamide-amide derived from (a) an unsaturated fatty acid with at least 12 carbon atoms or a dimer or polymer thereof and, (b) a polyalkylene-polyamine, and a further reaction product of (c) a polyepoxide compound and (d) a stoichiometric excess of a polyalkylene-polyamine, the additives being in finely divided form and added in an amount totalling 1 to 20%, preferably 1 to 12% by weight relative to the cellulose content in the spinning solution.

The nitrogen-containing additives employed in the process of this invention are known compounds, which can be incorporated into the viscose spinning solution in an aqueous medium, appropriately, with the aid of emulsifiers; they have good compatibility with the viscose.

To manufacture the amides containing amino groups; aliphatic, unsaturated monocarboxylic acids with at least 12 carbon atoms, preferably with 12 to 18 carbon atoms, such as oleic, linoleic, and linolenic acid, are used as component (a). Long chain unsaturated fatty acids containing hydroxyl groups, such as ricinoleic acid



are also suitable. The unsaturated fatty acids can also be used mixed with their dimerized, or polymerized derivatives, or the dimers or polymers may be used instead of the monomers. The polymerization of the acids probably takes place by a Diels-Alder mechanism, in that conjugated and, therefore, reactive carbon-carbon double bonds are produced in the unsaturated fatty acids by a partial or complete isomerization, these double bonds then completing the reaction to give a mixture of dimeric and higher polymeric fatty acids. Of course such a reaction can only take place if a starting material contains at least two conjugated carbon-carbon double bonds. With oleic acid, for example, it can only react if another compound having at least two conjugated double bonds is present.

Aliphatic polyamines with at least two primary or sec-

2

ondary amine groups, such as ethylenediamine, diethylenetriamine and triethylenetetramine, serve as component (b).

In addition to adding the polyamine-amide derived from components (a) and (b), it is required to add it to the viscose spinning composition with a further reaction product of a polyepoxide (c) and a stoichiometric excess of a polyalkylene-polyamine (d).

Suitable polyepoxides which may be used include the

10 polyglycidyl ethers such as those accessible by etherification of a dihydric alcohol or diphenol with epichlorohydrin in the presence of alkali. The epoxides which are obtained by reaction of bis(p-hydroxyphenyl)-dimethylmethane (Bisphenol A) with epichlorohydrin should be particularly mentioned. Reaction of these products with

15 the polyamines (d) then yields the second additive.

The polyamines (d) may be the same or similar to the amines which have been mentioned for component (b). The adduct of (c) and (d) contains no further free 20 epoxide groups since a stoichiometric excess of amine is always used.

The amounts of the components (a) to (d) which are reacted can vary within wide limits. Thus the amides containing amine groups may, for example, contain 40 to 80% 25 by weight of fatty acid or dimerized or polymerized fatty acid and 60 to 20% by weight of polyamine whilst the epoxide-amine compound is suitably derived from 25 to 40% by weight of an epoxide compound and 75 to 60% by weight of polyamine.

30 The additives (a) are added 90 to 10% by weight being a polyamine-amide derived from (a) and (b) and 10 to 90% by weight being a reaction product of (c) and (d).

In addition to the essential additions described above, 35 the reaction products may contain further additives, such as solvents and additional reagents such as epoxides and phenols.

The product of (a) and (b), mixed with a product of 40 (c) and (d), are suitably introduced in an aqueous medium into the viscose spinning solution. If the products are not water-soluble or only show limited solubility in water, an aqueous medium can be used which contains emulsifiers and/or organic solvents. The emulsifiers used can be anionic or cationic, but are preferably non-ionic. Suitable non-ionic emulsifiers include the addition products of 4 to 12 mols of ethylene oxide to long chain amines or alcohols with 12 to 24 carbon atoms or to alkylphenols with 10 to 18 carbon atoms. The emulsifiers are generally employed in amounts of between 1 and 20%, preferably between 1 and 5% by weight relative to the cellulose.

45 Suitable non-ionic emulsifiers include the addition products of 4 to 12 mols of ethylene oxide to long chain amines or alcohols with 12 to 24 carbon atoms or to alkylphenols with 10 to 18 carbon atoms. The emulsifiers are generally employed in amounts of between 1 and 20%, preferably between 1 and 5% by weight relative to the cellulose. The compounds and preparations intended for the manufacture of the viscose with novel dyeing properties can now be stirred directly in finely divided form into the spinning solution. The filtrability of the viscose is generally not adversely affected by the presence of the additives, so that

50 during the spinning process blocking of sieves mounted in front of the spinning nozzle arising from the presence of such additives, does not occur and a homogeneous filament material can be manufactured without fluctuations in gauge. The shaping of the viscose may be carried out in known manner, e.g. through spinnerets into a precipitation bath (e.g. a Muller bath) with optional post-treatment in further baths.

55 The fabrics and finished articles obtained from this viscose after the usual precipitation and shaping show good receptivity for dyestuffs which are not normally suitable for dyeing cellulosic materials. Suitable dyestuffs which can be employed are essentially all dyestuffs known for dyeing cellulosic materials; in addition, however, the large group of acid wool dyestuffs and dispersion dyestuffs, though these are normally only employed for dyeing nitrogen-containing fibres or polyester material, may 60 also be used.

Thus many useful dyestuffs can be used for dyeing cellulose material as a result of the process of this invention. These dyestuffs generally yield uniform and non-stripy dyeings with good fastness properties on the cellulosic material manufactured according to the invention.

Amongst the many known acid wool dyestuffs which can be used here, there may especially be mentioned the metal-containing dyestuffs such as 1:2-chromium or cobalt complex dyestuffs, the dyestuff molecule of which can contain free acid groups conferring solubility in water, or 1:1 metal complex dyestuffs. Of the dispersion dyestuffs, azo and anthraquinone dyestuffs should particularly be mentioned.

The cellulose material manufactured according to this invention behaves particularly well in a mixture with, for example, untreated cellulosic fibres. Here it is possible to achieve, with a dyestuff mixture of a direct dyestuff and wool dyestuff, applied from a single dyebath, dyeing effects and color patterns which are determined by the fibre distribution (for example strips of any desired width and any desired spacing) in the mixed fabric. The direct dyestuff dyes the entire fabric whilst the wool dyestuff only dyes the fibres in the fabric which has been manufactured according to the invention (differential dyeing).

Tone-in-tone dyeings of fibre mixtures of the fibre material according to the invention and wool/polyamides or polyester fibre material can be obtained using wool or dispersion dyestuff.

The dyeing of the material may be carried out in the usual manner for these dyestuffs, for example, according to the padding process or the exhaustion process at an elevated temperature.

The essential advantage of the cellulose material manufactured according to this invention resides in the fact it remains cellulose like and, nevertheless, possesses the novel dyeing properties described. It thus differs from the so-called "animalized" cellulosic fibres which are obtained from viscose spinning composition into which large amounts of nitrogen-containing substances are incorporated. These animalized cellulosic fibres have partially

lost the dyeing properties of cellulose and in this respect behave more like wool.

The following examples further illustrate the present invention. Unless otherwise stated, the parts quoted in the example are parts by weight.

#### EXAMPLE I

5 g. of the preparation A described below are emulsified with 5 g. of an addition product of 8 mols of ethylene oxide to 1 mol of p-tert-octylphenol, filtered and stirred into 983 g. of viscos (75 g. of cellulose). The viscose is spun in the usual manner with the aid of a precipitation bath containing sulphuric acid to give long fibres. The fibres are subsequently washed in after-treatment baths (for example water), desulphurized (for example with dilute aqueous solutions of sodium sulphide and sodium hydroxide) washed and brightened.

Preparation A consists of 28.6 parts of a Component I and 71.4 parts of a Component II. Component I is manufactured as follows: A reaction mixture of 48.2 parts of diethylenetriamine, 34.6 parts of bisphenol A and 17.2 parts of a bisphenol A-epichlorohydrin resin with 182 to 191 epoxide equivalents per kg. of resin is reacted for about 5 hours at 200° C., with the volatile constituents being distilled off towards the end of the reaction by applying a water pump vacuum.

Component II is manufactured as follows: A mixture of 40 parts of tall oil fatty acid and 13.8 parts of dimerised fatty acids is heated to 130° C. whilst stirring and is mixed with 34 parts of triethylenetetramine at this temperature. The temperature is then raised to 200° C. and is kept for 3 hours at this value, with a water pump vacuum being applied in the last hour.

The resulting polyamine-amide is then further mixed with 17.2 parts of xylene.

The cellulose material manufactured with this preparation can be well dyed with acid wool dyestuff and dispersion dyestuffs according to the methods known for dyeing with these dyestuffs. Suitable dyestuffs are, amongst others:

#### 1:2-chromium complex



Reddish brown:

#### 1:2-cobalt complex



Yellow.

#### 1:2-chromium complex



Orange:

| 1:2-chromium complex |                      |         |
|----------------------|----------------------|---------|
| (4).....             |                      | Red.    |
|                      | 1:2-cobalt complex   |         |
| (5).....             |                      | Claret. |
|                      | 1:2-cobalt complex   |         |
| (6).....             |                      | Violet: |
|                      | 1:1-chromium complex |         |
| (7).....             |                      | Blue:   |
|                      | 1:1-chromium complex |         |
| (8).....             |                      | Yellow. |
|                      | 1:1-chromium complex |         |
| (9).....             |                      | Pink.   |
|                      | 1:1-chromium complex |         |
| (10).....            |                      | Blue:   |
|                      | 1:1-chromium complex |         |

These dyestuffs yield nonstriped dyeings with good fastness properties on the cellulose material manufactured according to the invention. In comparison to polyamide and wool material which has been dyed with the wool dyestuff mentioned or in comparison with polyester material which has been dyed with the dispersion dyestuffs mentioned, the cellulose material according to the invention shows a tone-in-tone dyeing.

#### EXAMPLE 2

7.5 g. of the Preparation B described below are filtered in the form of a 20% strength aqueous solution and stirred into 983 g. of viscose (75 g. of cellulose).

The viscose is spun as described in Example 1 and the fiber material is appropriately after-treated. Preparation B is manufactured as follows:

A solution of 49.4 g. of a condensation product of polymerized linoleic acid and diethylenetriamine having an amine equivalent of 247, and 49.4 g. of methanol, are

added over the course of 24 minutes, with good stirring, into a solution, warmed to 51° C., of 38.4 g. of an epoxide formed from 4,4'-dihydroxydiphenyl-2,2'-propane and epichlorhydrin, having an epoxide equivalent of 191, and 38.4 g. of methanol, the reaction temperature being 51 to 53° C. 3 g. of glacial acetic acid are added after 8 minutes and again after 18 minutes from the start of the dropwise addition, and after 24 minutes a further 2 g. of glacial acetic acid are added. The reaction is continued for a further 2 hours and 35 minutes at 55 to 60° C. The reaction product is then soluble in water to form an opalescent solution. Thereafter 4 g. of glacial acetic acid and 273.4 g. of water are added whilst stirring. A yellowish viscous cloudy 20% solution having a pH-value of 5.2 is obtained.

A mixed cellulosic fabric of viscose fibres and fibres manufactured according to the invention with Preparation B, the latter having been woven in as stripes, is dyed by

the exhaustion process, in a known manner, with the following dyestuffs:



A fast blue dyeing with violet stripes is obtained.

We claim:

1. A process for the manufacture of viscose fibers with novel dyeing properties, which comprises adding to the viscose spinning solution before precipitation from 1 to 20% by weight, based on the weight of cellulose content in said spinning solution, of a mixture comprising:
  - (A) from 90 to 10% by weight of a polyamine-amide obtained by reacting (a) from 40 to 80% by weight of an unsaturated fatty acid with at least 12 carbon atoms or a dimer or polymer thereof and, (b) from 20 to 60% by weight of a polyalkylene-polyamine; and
  - (B) from 10 to 90% by weight of a polyepoxide-polyamine product obtained by reacting (c) from 25% to 40% by weight of a polyepoxide and (d) a stoichiometric excess of a polyalkylene-polyamine, said polyalkylene-polyamine being present in an amount of from 75 to 60% by weight.

2. A process according to claim 1 wherein (a) is an unsaturated fatty acid with 12 to 18 carbon atoms or a dimer or polymer thereof.
3. A process according to claim 1 wherein (c) is a reaction product of Bisphenol A and epichlorohydrin.
4. A process according to claim 1 wherein (b) and (d) is ethylenediamine, diethylenetriamine or triethylenetetramine.
5. A process according to claim 1 wherein the additives derived from (a) and (b) and from (c) and (d) are added to the spinning solution as an aqueous or organic solution or a dispersion.
6. A process according to claim 5 wherein the additives are added to the spinning solution in the presence of a non-ionic emulsifier.
7. A process according to claim 1 wherein the additives are added 90 to 10% by weight being a polyamine-amide derived from (a) and (b) and 10 to 90% by weight being a reaction product of (c) and (d).
8. A process according to claim 1 wherein the additives are added in an amount totalling 1 to 12% by weight based on the cellulose content in the spinning solution.

#### References Cited

##### UNITED STATES PATENTS

|           |         |                  |         |
|-----------|---------|------------------|---------|
| 2,767,089 | 10/1956 | Renfrew et al.   | 260—21  |
| 2,852,334 | 9/1958  | Hollihan et al.  | 264—144 |
| 2,971,816 | 2/1961  | Hollihan et al.  | 264—193 |
| 3,016,305 | 1/1962  | Vosfers          | 106—165 |
| 3,046,085 | 7/1962  | Burroughs et al. | 264—194 |
| 3,066,032 | 11/1962 | Fukushima et al. | 106—165 |
| 3,106,444 | 10/1963 | Mueller          | 264—194 |
| 3,278,560 | 10/1966 | Garbner          | 8—116.2 |

##### FOREIGN PATENTS

|          |         |       |         |
|----------|---------|-------|---------|
| 37-17771 | 10/1962 | Japan | 264—188 |
|----------|---------|-------|---------|

JAY H. WOO, Primary Examiner

U.S. CL. X.R.

40 106—165, 170, 186; 260—13; 264—194, 191



1. A process for the manufacture of viscose fibers with novel dyeing properties, which comprises adding to the viscose spinning solution before precipitation from 1 to 20% by weight, based on the weight of cellulose content in said spinning solution, of a mixture comprising:
 

- (A) from 90 to 10% by weight of a polyamine-amide obtained by reacting (a) from 40 to 80% by weight of an unsaturated fatty acid with at least 12 carbon atoms or a dimer or polymer thereof and, (b) from 20 to 60% by weight of a polyalkylene-polyamine; and
- (B) from 10 to 90% by weight of a polyepoxide-polyamine product obtained by reacting (c) from 25% to 40% by weight of a polyepoxide and (d) a stoichiometric excess of a polyalkylene-polyamine, said polyalkylene-polyamine being present in an amount of from 75 to 60% by weight.

2. A process according to claim 1 wherein (a) is an unsaturated fatty acid with 12 to 18 carbon atoms or a dimer or polymer thereof.

3. A process according to claim 1 wherein (c) is a reaction product of Bisphenol A and epichlorohydrin.

4. A process according to claim 1 wherein (b) and (d) is ethylenediamine, diethylenetriamine or triethylenetetramine.